

## UNITED STATES PATENT OFFICE

2,487,906

## IGNITION COMPOSITION

William D. Trevorow, Hometown, Pa., assignor to  
 Atlas Powder Company, Wilmington, Del., a  
 corporation of Delaware

No Drawing. Application July 8, 1946,  
 Serial No. 682,155

6 Claims. (Cl. 52—4)

1

The present invention relates to compositions of matter for the preparation of ignition devices.

An object of the present invention is the provision of a composition of matter of the type specified which does not tend to jell.

Another object of the invention is the provision of a composition of matter of the type specified which has desirable viscosity characteristics.

Other objects of the invention will be apparent from the following description.

Ignition devices are customarily prepared by surrounding heatable elements such as an electric bridge wire with a coating composition carrying a heat-sensitive ignition compound.

One common type of igniter is the bridge plug type used in some forms of electric detonators. A bridge plug comprises a plug of material separating two leg wires connected together by a fine, high resistance, bridge wire. A coating composition, admixed with an ignition compound, is spread around the bridge wire. The spreading operation is called buttering because of the viscous consistency of the composition containing the ignition compound. The buttered material dries hard on evaporation of the solvent, and subsequent heating of the bridge wire as by passage of an electric current fires the ignition material with the production of a burst of flame.

Another form of igniter, also commonly used in detonators, is the electric match which is composed of two insulated metal plates or foils connected together by a bridge wire and dipped in a coating composition containing an ignition compound. The dipping operation forms, around the bridge wire, a drop of ignition material which hardens on drying. Electric matches also may be fired by passage of an electric current through the bridge wire.

While many different materials are used for ignition compounds, lead salts of nitrophenols have been found particularly desirable in many instances. Examples of lead nitrophenols which are particularly useful in accordance with the present invention are lead styphnate, monobasic lead 4:6 dinitro-ortho-cresylate, monobasic lead picramate, monobasic lead 3:5 dinitro-benzoate, lead nitroato-bis-basic-lead 4:6 dinitro-ortho-cresylate, normal lead 2 nitro-resorcinate and monobasic lead 2 nitro-resorcinate.

The coating composition which is used to carry the ignition compound is usually of the lacquer type composed of a highly combustible nitrocarbohydrate such as nitrostarch or nitrocellulose and a volatile solvent such as esters of the type of butyl acetate and amyl acetate, aromatic hy-

drocarbons such as benzene, and the like. Depending on the viscosity or volatility characteristics desired, different solvents or mixtures of solvents are used as is well understood in the art.

5 A difficulty which has been found to occur when lead salts of nitrophenols are used in lacquers of this type has been that the composition tends to set up into a gel prior to use, and in a gel form it is difficult to apply.

10 According to the present invention, it has been discovered that compositions of the present type do not exhibit this gelling phenomenon when acetone or acetonyl acetone are included in them. Either or both of these materials has been found 15 to be successful.

Acetonyl acetone is usually somewhat to be preferred, particularly when the compositions are to be used for operations of the buttering type. When buttering mixtures are prepared, it is customary to originally prepare them in thin form and then to evaporate them to the desired viscous consistency which makes for easy buttering. When acetone is used in such mixtures it sometimes volatilizes away before the composition is 20 thick enough for use. Acetonyl acetone does not 25 show this disadvantage.

When the compositions can be used in less viscous form, as for dipping, acetone is found to be entirely satisfactory.

30 While acetone and acetonyl acetone may be used as sole solvents, it is usually preferred that they be used in proportions of from about 1 to about 20% by volume based on the total volume of the composition excluding ignition compounds.

35 The following example is illustrative of a specific embodiment of the invention:

A lacquer was made up by adding 2.4% by weight of nitrostarch to a solvent which was composed of 95% butyl acetate and 5% benzene. 180

40 cc. of this lacquer were mixed with 200 grams of lead styphnate and 20 cc. of acetonyl acetone. This mixture was partially dried until it became viscous and then was buttered on to the bridge wires of bridge plugs. At no time did the composition exhibit any jelling tendency and it buttered readily. After drying, the igniters produced 45 were found to be entirely satisfactory.

A composition particularly suitable for the preparation of match heads may be made by using

50 a lacquer composed of nitrocotton dissolved in amyl acetate and by substituting acetone for acetonyl acetone. As is well understood in the art, it is usually desirable to protect match heads by dips of protective coating. A first protective dip 55 of a 6 oz. ether alcohol nitrocotton lacquer, and

a second protective dip of a 6 oz. amyl acetate nitrocotton lacquer are quite satisfactory for the purpose.

What is claimed is:

1. A composition of matter comprising nitro-starch, a volatile solvent therefor, an anti-gelling agent selected from the class consisting of acetone and acetyl acetone and an ignition compound selected from the group consisting of lead styphnate, monobasic lead 4:6 dinitro-ortho-cresylate, monobasic lead picramate, monobasic lead 3:5 dinitro-benzoate, lead nitro-bis-basic-lead 4:6 dinitro-ortho-cresylate, normal lead 2 nitro-resorcinate and monobasic lead 2 nitro-resorcinate, said anti-gelling agent comprising from about 1 to about 20% by volume of the composition exclusive of ignition compound.

2. A composition of matter comprising nitrocotton, a volatile solvent therefor, an anti-gelling agent selected from the class consisting of acetone and acetyl acetone, and an ignition compound selected from the group consisting of lead styphnate, monobasic lead 4:6 dinitro-ortho-cresylate, monobasic lead picramate, monobasic lead 3:5 dinitro-benzoate, lead nitro-bis-basic-lead 4:6 dinitro-ortho-cresylate, normal lead 2 nitro-resorcinate and monobasic lead 2 nitro-resorcinate, said anti-gelling agent comprising from about 1 to about 20% by volume of the composition exclusive of ignition compound.

3. A composition of matter comprising lead styphnate, butyl acetate, benzene, acetyl acetone, and nitrostarch.

4. A composition of matter comprising a nitro-carbohydrate in solution, acetyl acetone as an anti-gelling agent and an ignition compound selected from the group consisting of lead styph-

nate, monobasic lead 4:6 dinitro-ortho-cresylate, monobasic lead picramate, monobasic lead 3:5 dinitro-benzoate, lead nitro-bis-basic-lead 4:6 dinitro-ortho-cresylate, normal lead 2 nitro-resorcinate and monobasic lead 2 nitro-resorcinate, said anti-gelling agent comprising from about 1 to about 20% by volume of the composition exclusive of ignition compound.

5. A composition of matter comprising a combustible nitrocarbohydrate, a volatile solvent therefor, an anti-gelling agent selected from the class consisting of acetone and acetyl acetone, and an ignition compound selected from the group consisting of lead styphnate, monobasic lead 4:6 dinitro-ortho-cresylate, monobasic lead picramate, monobasic lead 3:5 dinitro-benzoate, lead nitro-bis-basic-lead 4:6 dinitro-ortho-cresylate, normal lead 2 nitro-resorcinate and monobasic lead 2 nitro-resorcinate, said anti-gelling agent comprising from about 1 to about 20% by volume of the composition exclusive of ignition compound.

10 6. A composition of matter according to claim 5 in which said anti-gelling agent is acetyl acetone.

15 20 25 WILLIAM D. TREVORROW.

#### REFERENCES CITED

The following references are of record in the file of this patent:

#### UNITED STATES PATENTS

| Number    | Name       | Date          |
|-----------|------------|---------------|
| 1,045,012 | Flursheim  | Nov. 19, 1912 |
| 1,964,077 | Piccard    | June 26, 1934 |
| 2,159,229 | Rubenstein | May 23, 1939  |